

## UNITED STATES PATENT OFFICE.

JOSEPH T. VAN DER GRACHT, OF CAMPBELL, CALIFORNIA.

## ARTIFICIAL PARCHMENT AND METHOD OF MAKING THE SAME.

No Drawing.

Application filed March 15, 1922. Serial No. 544,020.

*To all whom it may concern:*

Be it known that I, JOSEPH T. VAN DER GRACHT, a subject of the Queen of the Netherlands, residing at Campbell, in the county 5 of Santa Clara, State of California, have invented a new and useful Artificial Parchment and Method of Making the Same, of which the following is a specification.

My invention relates to the art of making 10 artificial parchment. Parchment, which is prepared skin, has been used from time immemorial where great permanence or wearing qualities were desired, it being a common practice to engross important documents upon parchment which has been especially prepared therefor.

Parchment is open to certain objections. Since it is built up entirely of animal tissues and their included greases it is extremely 20 susceptible to atmospheric conditions, warping, shrinking and becoming very brittle with age as may be easily seen from an inspection of the binding of old books or from an inspection of sheets of old 25 manuscript.

The principal object of my invention is to produce an artificial parchment which will have many of the good qualities of the genuine parchment with few of its disadvantages and which will closely resemble 30 parchment in appearance.

This artificial parchment is prepared in the following manner:

I prefer to use as a base Japanese vellum 35 or a similar paper which is first thoroughly soaked in cold water. As a result of this soaking, some portions of the paper, which are more absorbent than others, are more thoroughly saturated with the water than 40 the remainder of the paper. The saturated paper is then spread out upon a sheet of blotting paper or cloth or some other absorbent substance and is covered by a layer of such absorbent substance for the 45 purpose of partially drying out the paper and particularly for removing superfluous water therefrom.

The moistened paper is then covered with a varnish which is applied with a 50 brush. The varnish must be free from oil and is preferably irregularly applied so that a considerable quantity is used on certain portions of the paper and only a very light coating on the remainder. The portions 55 of the paper which have been most

thoroughly saturated with water take the varnish more readily than less water saturated parts since they are more porous. The result is that the coat of varnish is somewhat irregular, a portion of the paper 60 having a heavy coating whereas the remainder has only a light coating. This gives the paper the appearance of natural parchment, the degree of resemblance depending upon the skill of the workman. 65 The paper is then allowed to dry and, when dried, has the stiff and brittle feeling of natural parchment.

If it is desired to produce an old parchment effect, the dark blotches of the old 70 parchment may be produced by graphite which is rubbed into the paper before soaking.

While I prefer to use a Valspar varnish, it should be understood that there are several resinous materials which may be used if dissolved in a suitable evaporative solvent such as alcohol.

The final product consists of the cellulose of the paper which is imbedded in and 80 protected by the resinous material. It is a well known fact that Egyptian papyrus, which is a long fibered paper, has given proof that a pure cellulose paper is extremely long lived. It is also a well known 85 fact that cloth or paper which is thoroughly impregnated with resinous material is also extremely long lived, the impregnated cloth wrappings of the Egyptian mummies being found practically unchanged after long 90 periods of time.

I have found that the artificial parchment produced by me may be used without treatment for ordinary printing purposes due to the fact that it is free from grease 95 and will take any standard ink without being treated beforehand as is necessary where real parchment is used. Such artificial parchment also takes both water and oil colors without preparation and may be used 100 for bookbinding without such preparation.

Obviously, an artificial parchment of this type can be produced at a small cost as compared to natural parchment, but the principal advantages of my invention reside in the greater efficiency and durability of the product as compared to real parchment. The long fiber Japanese paper, preferably used by me, is very tough and the varnish 105 greatly improves its strength and hardness 110

so that it will resist the surface wear. At the same time, the varnish, if properly applied, robs the paper of none of its flexibility.

5 I claim as my invention:

1. A process of producing an artificial parchment which comprises soaking a paper in water and distributing resinous material over the surface of said paper while said

10 paper is still wet.

2. An artificial parchment consisting of vellum paper having its fibres imbedded in, and protected by, oil-free varnish material irregularly distributed therethrough, said

artificial parchment resembling natural 15 parchment in appearance.

3. An artificial parchment consisting of long-fibre vellum paper initially capable of an irregular absorption of moisture and having its fibres imbedded in and protected 20 by oil-free varnish irregularly distributed over it, said artificial parchment resembling natural parchment in appearance.

In testimony whereof, I have hereunto set my hand at San Francisco, California, 25 this 2nd day of March, 1922.

JOSEPH T. VAN DER GRACHT.